

June 5, 1923.

1,457,453

P. A. MURPHY

DRAWING ROLL

Filed May 25, 1922



Inventor:  
Patrick A. Murphy,  
by his attorney,  
Charles S. Gooding.

## UNITED STATES PATENT OFFICE.

PATRICK A. MURPHY, OF LYNN, MASSACHUSETTS, ASSIGNOR TO TEXTILE RUBBER CO., OF BOSTON, MASSACHUSETTS, A CORPORATION OF MASSACHUSETTS.

## DRAWING ROLL.

Application filed May 25, 1922. Serial No. 563,514.

To all whom it may concern:

Be it known that I, PATRICK A. MURPHY, a citizen of the United States, residing at Lynn, in the county of Essex and State of Massachusetts, have invented new and useful Improvements in Drawing Rolls, of which the following is a specification.

This invention relates to drawing rolls for spinning machines.

10 For many years it has been the practice in the textile industry to equip the various types of spinning machines which employ drawing rolls with top rolls having an outer covering composed of leather and while many attempts have been made to provide a substitute for said leather, and top drawing rolls have been constructed with coverings composed of certain fabrics treated with various materials, to my knowledge 20 none of these rolls have proved successful and no rolls have ever been constructed which have proved practical with a covering consisting entirely of a rubber compound.

25 In leather rolls there is invariably a space between the abutting ends of the leather and often the thickness of said leather varies to such an extent that it is difficult to construct a perfectly accurate roll. Leather also deteriorates quickly being easily affected by oil, especially present in woolen yarn. Moreover in all cotton and woolen mills the atmosphere is kept moist by employing humidifiers in large numbers and the atmosphere is at all times saturated with said moisture which has a bad effect upon the leather often causing the same to become detached from the metal core of the roll to which it is attached by an adhesive material.

30 The object of the present invention therefore is to so construct a top drawing roll that all of the above objections will be eliminated, the roll produced being perfectly accurate and free from seams and crevices and composed of materials not easily affected by the before-mentioned conditions and at the same time greatly reducing the cost of the rolls.

35 The invention consists in the construction of drawing rolls as set forth in the following specification and particularly pointed out in the claims thereof.

Referring to the drawings:

55 Figure 1 represents a sectional elevation

of a portion of a spinning frame illustrating a general type of machine employing rolls embodying my invention.

Fig. 2 is a front elevation partly broken away and illustrated in section of a top drawing roll embodying my invention.

Like numerals refer to like parts throughout the several views of the drawings.

In the drawings, 5 represents a portion of a frame of a spinning machine of well known type upon which are rotatably mounted a top drawing roll 6 and a fluted metallic drawing roll 7. The top roll 6 rests upon the roll 7 and is driven by frictional contact with the latter roll. A plurality of strands 8 of material composed of very loosely assembled cotton, silk or woolen fibers are fed between a plurality of guide rolls 9, 10, 11 and 12 by which they are loosely joined into a single strand 13 which then passes between rolls 14 and 15, thence over a roll 16 and between the drawing rolls 6 and 7.

A spool 17 rests upon a table 18 upon which it is raised and lowered and also rotated by mechanism not shown but well known to those skilled in the art, and a spindle 19 extends vertically through said spool and has a flier 20 attached thereto. The spindle 19 and flier 20 are rotated very rapidly by mechanism not shown and also well known to those skilled in the art, and the fibers of the strand 13 which before it passes through the rolls 6 and 7 consists of several strands 8 loosely united, are simultaneously merged and drawn into a smaller and more compact strand 21 and wound upon the spool 17.

All the mechanism thus far described is old and well known in the art and the novelty of the present invention resides in the construction of the top drawing roll 6 and particularly in a material used as a covering for said roll, the latter being of such a character that the strand may pass between the rolls 6 and 7 without danger of the delicate fibers of which it is composed being crushed or broken.

The roll 6 is constructed with a rigid core or boss 22 preferably composed of metal and having grooves extending around its periphery upon which is placed a comparatively thin layer of a suitable rubber compound 23 which becomes very hard when cured and which very tightly adheres to the

periphery of the metal core 22. The layer 23 is placed upon the core 22 in a plastic state and is evenly distributed around the periphery thereof after which a layer 24 of 5 suitable thickness of another rubber compound is placed upon the layer 23. The materials of which the layer 24 is composed are as follows:—14 pounds Ceylon rubber, 3 pounds black rubber shoddy, 12 pounds 10 blue lead, 4 pounds litharge,  $3\frac{1}{2}$  pounds fine asbestos, 3 pounds lime and  $2\frac{1}{2}$  pounds of sulphur. After being prepared in the usual well known manner the composition in a plastic state is placed in a mass around the 15 layer 23, and the core with the superimposed layers 23 and 24 thereon is then placed in a mould and subjected to heat at a temperature of from  $150^{\circ}$  to  $200^{\circ}$  for a period of from one and one quarter hours to one and 20 one-half hours during which period the composition is cured, thereby rendering the inner layer 23 very hard and the outer layer 24 sufficiently hard to be durable yet at the same time retaining a sufficient resiliency for 25 the purpose required. After being taken from the mould the periphery of the roll is finished so that the roll will be perfectly cylindrical and the periphery of said roll being perfectly smooth and free from cracks and 30 seams will not injure the most delicate fibers.

The layer of hard rubber 23 is utilized as a medium for fastening the outer layer 24 to the core 22 to prevent said layer from creeping thereon, it having been found that while 35 it is possible to secure the layer 24 directly to the core, there is a tendency for said layer to loosen after long continued use, whereas the layer 23 when cured, adheres to the core so tightly that there is no danger of it ever 40 becoming loosened, and during the curing process, the adjacent surfaces of the layers 23 and 24, in effect, unite and form a single mass.

The material of the covering 24 as above 45 constructed has been found very durable, is not affected by the oil present in woolen yarns and is impervious to the moisture in the room, being benefited by said moisture rather than being injured thereby. By actual test it has been found that by using my 50 improved roll a better quality of yarn may be produced, said yarn being drawn much more evenly and at the same time produc-

ing a greater yardage than is possible with rolls having a leather covering. Moreover 55 the cost of producing rolls in accordance with my invention is much less than the cost of producing leather covered rolls and the rubber rolls will last very much longer than the leather rolls.

It has also been found when rolls are used constructed in accordance with this invention, that much less power is required to drive the machine upon which they are employed for the reason that it is not necessary 60 to force the top drawing roll 6 against the lower drawing roll 7 with as much pressure to obtain the necessary gripping effect as is the case with leather covered rolls.

I claim:

1. A drawing roll having, in combination, a rigid core and a plurality of superimposed layers of rubber compound located upon said core, the degree of hardness of said layers decreasing from the inner layer outward.

2. A drawing roll having, in combination, a rigid core, a layer of hard rubber compound surrounding said core and a second layer of rubber compound surrounding 80 said first layer and consisting of Ceylon rubber, black rubber shoddy, blue lead, litharge, fine asbestos, lime and sulphur, said layers being moulded and cured upon said core to produce a softer layer than said first-named layer.

3. A drawing roll having, in combination, a rigid core, a layer of hard rubber compound surrounding said core and a second layer of rubber compound surrounding 90 said first layer and embodying the following materials in the following proportions, 14 pounds of Ceylon rubber, 3 pounds of black rubber shoddy, 12 pounds blue lead, 4 pounds litharge,  $3\frac{1}{2}$  pounds fine asbestos, 3 pounds of lime and  $2\frac{1}{2}$  pounds of sulphur, said layers being moulded and cured upon said core to produce a softer layer than said first named layer.

In testimony whereof I have hereunto set 100 my hand in presence of two subscribing witnesses.

PATRICK A. MURPHY.

Witnesses:

FRANKLIN E. LOW,  
HAZEL F. LA MUDGE.